

## UNITED STATES PATENT OFFICE

2,107,146

## BURNING BRICK

Thomas B. Dreher, Pottsville, Pa.

No Drawing. Application February 24, 1937,  
Serial No. 127,402

8 Claims. (Cl. 25—157)

This invention relates to improvements in methods of producing black brick and other ceramic products.

Manufacturers have long tried to make black brick by different methods but no quantity of satisfactory brick was produced by these methods. One of these previous methods included coating bricks with manganese compounds or mixing manganese compounds with the clay before burning. Another method was known as "flashing". In these treatments to produce black brick, the manufacturers always maintained too high a temperature in the kiln to get the desired results.

According to my invention I produce brick in commercial quantities which is black on all faces and through and through. To produce these black bricks, I finish burning the brick in the usual way and then reduce the temperature to about 1200° F. or to about  $\frac{1}{2}$  of the normal burning temperature used in manufacturing brick. Then I fill up the fire boxes with soft coal with as high a volatile content as obtainable and burn the soft coal with an insufficient supply of air in order to produce large quantities of smoke. This smoke is circulated through the kiln. When all the smoke has burned out of the soft coal or the coal has coked, part of the coke is removed and more soft coal is added and this operation is repeated until a sample taken out and cooled shows that the brick is black. Then the fire is raked out as fast as possible and the brick is cooled quickly. The resulting product is a black brick which is black on all faces and through and through. Instead of soft or bituminous coal I may use other coals or fuels which form heavy or black smoke when insufficient air is supplied for combustion, as for example, fuel oil.

My invention will now be more specifically set forth. My process of producing black brick starts with the brick which is still hot after the usual burning operations. That is, the brick is finished by burning in any of the usual ways and my process starts here at the completion of the burning and while the brick is at the high temperature of about 1500° F. to 1950° F. I start by cutting off the supply of fresh fuel to the fire boxes and allowing cold air to pass over the fires into the kiln. Any other method of cooling the kiln may be used. Sufficient fire is kept in the furnaces to ignite the soft coal which is later added when the kiln is ready for the smoking operation.

When the temperature of the kiln and brick has been reduced to about 900° F. or not over 1200° F. the fire boxes are filled up with bi-

tuminous coal and as each fire gets under way, the draft below the grate is shut off and very little or no air is allowed to pass over the top of the fire. The damper in the stack or stacks is lowered or the draft is shut off sufficiently to draw the smoke only from the furnaces and circulate it very slowly through the kiln and in contact with the hot brick.

When all the smoke has burned out of the coal or fuel or the coal is coked, part of the hot coke is raked from the fires but sufficient hot coke is left in the fire boxes to ignite a new batch of bituminous coal or fuel which is then added. After this new batch of coal is coked, the operation of removing part of the coke and coaling up the fires with bituminous coal is repeated as often as necessary to insure smoking the brick to complete blackness throughout. In certain instances it will take about 70 hours of smoke treatment to obtain my black brick product. This time of treatment may be varied within limits to suit different conditions or to produce slightly different effects.

During the smoking treatment the temperature of the brick and kiln may rise from about 900° F. or about 1200° F. to not over about 1400° F. When the smoking period is completed, the fire in all the fire boxes is raked out or removed as quickly as possible. Then the kiln doors are opened partly and after the doors have been open for about two hours and the temperature of the brick reduced to about 1100° F., a blower is put in front of one door and air is blown into the kiln to blow the hot air out. This is continued until no red hot brick can be seen and until the temperature of the brick is reduced to about 500° F. The blower will normally be in operation about 8 hours. In some instances the kiln doors may be opened wide at the beginning of the cooling operation to obtain faster initial cooling. Any method of quick cooling may be used that will not damage the product.

The brick is then removed from the kiln in the usual manner and the brick produced are black on all the faces and through and through.

In my method it is important to reduce the temperature of the burned brick before proceeding with the smoking treatment and it is also important to rapidly cool the brick after the smoking treatment. This latter cooling is done more quickly than the usual methods of cooling after burning brick in the usual ways. Generally after completion of the smoking operation the brick is cooled from about 1400° F. to about 500° F. in about 10 to 12 hours.

5

10

15

20

25

30

35

40

45

50

55

As above set forth, my method starts with brick immediately after the burning has been finished in the usual ways. This method applies to and is effective in making black brick regardless of the mineral contents of which the brick is made. Any material that can be burned into brick or ceramic products can be turned black by this process. An analysis of one example of ordinary brick made by usual methods will now be given but it is to be expressly understood that the same does not form part of my invention, nor is my invention to be restricted thereto as the example is merely included to give one method of burning brick preparatory to the application of my process thereto. Other brick mixtures may be used and other temperatures used, it being only necessary that the burning of the brick be substantially completed.

|            | Per cent |
|------------|----------|
| 20 Silica  | 61.35    |
| Iron       | 10.16    |
| Aluminum   | 26.46    |
| Lime       | 0.32     |
| Magnesium  | 0.71     |
| 25 Sulphur | 0.20     |

The brick is stacked into a kiln and the fire started. The kiln is fired until the finishing temperature is obtained and this temperature is maintained as long as necessary to complete the burn. After the brick is burned, the temperature of the brick and kiln is reduced to about 900° F. or not over 1200° F. The brick is then ready for my process and is treated in the way as above given.

Brick or similar material burned in other ways may be treated according to my method to produce black brick or the like. The temperatures given by me may be varied within limits and also the smoking period may be varied.

When the smoking is completed and the kiln is cooled sufficiently to handle the brick, they are ready for sale or shipments. There is practically no soot deposit on the brick when finished smoking, and not any more than when the brick is burned in the usual method. The brick are black through and through and all faces are jet black.

If salt glazed brick are desired, it is only necessary to mix with the fuel each time the smoke fire is renewed, approximately six (6) pounds of coarse salt to each fire box, and smoke in the same manner as described for jet black brick. This method will produce a glazed or glossy black brick.

It is to be understood that the foregoing example is given only by way of illustration and that the same may be modified in many particulars without departing from the spirit of my invention, and my invention applies to ceramic products made by any of the different processes of manufacture, such as stiff mud, soft mud, hand made or any other process. The wood brick or brick product is used throughout merely for the sake of brevity.

What I claim is:

1. A method of the character described for producing black brick which comprises cooling brick in a kiln from the burning high temperature to about one-half the burning high temperature, subjecting the cooled brick to an extended

period of smoking, and then cooling the smoked brick quickly.

2. A method of the character described for producing black ceramic articles which comprises cooling ceramic articles in a kiln from the burning temperature to a lower temperature, subjecting such articles to a smoky atmosphere for an extended period of time, and then cooling the smoked articles quickly. 5

3. A method of the character described for producing black brick which comprises cooling brick in a kiln from the finishing temperature to about 900° F. or not higher than 1200° F., subjecting such brick to freshly formed smoke from burning bituminous fuel with an insufficient supply of air 15 for complete combustion, continuing the smoke treatment of the brick for a period sufficient to produce black brick and then cooling the smoked brick quickly. 10

4. A method of the character described for producing black brick which comprises providing brick at about 900° F. and not above 1200° F. in a confined space, subjecting such brick to a smoky atmosphere for an extended period of time, circulating the smoky atmosphere in the confined 25 space, and then cooling the smoke brick by reducing the temperature quickly from the very beginning of the cooling operation after smoking.

5. A method of the character described for producing black brick which comprises providing 30 burned brick at about 1100° F. to about 1200° F. in a confined space, subjecting such brick for an extended period of time to hot smoke freshly formed by burning bituminous coal with a supply of air insufficient for complete combustion, 35 circulating the smoke in such confined space in contact with the brick, and then cooling the smoked brick by quickly reducing the temperature at the beginning of the cooling operation.

6. A method of the character described for 40 producing black brick which comprises cooling brick in a kiln from the burning temperature to a substantially lower temperature, subjecting such brick to a smoky atmosphere for an extended period of time, and then cooling the smoked 45 brick quickly.

7. A method of the character described for producing black brick which comprises providing burned brick at about 1100° F. to about 1200° F. in a confined space, subjecting such brick for an 50 extended period of time to hot smoke, circulating the smoke in such confined space in contact with the brick, and then cooling the smoked brick by quickly reducing the temperature thereof. 55

8. A method of the character described for producing black brick which comprises cooling brick in a kiln from the finishing temperature to about 900° F., or not higher than 1200° F., subjecting such brick to freshly formed smoke from burning bituminous fuel with an insufficient supply of air 60 for complete combustion, continuing the smoke treatment of the brick in a rising temperature whose limit is 1400° F. for a period sufficient to produce black brick, and then cooling the smoked brick quickly from the highest temperature reached by said brick during the smoking operation. 65

THOMAS B. DREHER. 70